

## UNITED STATES PATENT OFFICE

2,095,975

## MAGNESIUM ALLOYS

Edward F. Fischer, Cleveland, Ohio, assignor, by  
mesne assignments, to Magnesium Develop-  
ment Corporation, a corporation of Delaware

No Drawing. Application August 7, 1935,  
Serial No. 35,126

3 Claims. (Cl. 75—168)

This invention relates to wrought magnesium base alloys and it is particularly concerned with those alloys which contain from about 5 to 10 per cent aluminum, 0.1 to 1 per cent manganese, 5 0.05 to 0.05 per cent calcium, and 0.1 to 1.5 per cent zinc.

Magnesium base alloys containing aluminum and zinc have proved to be quite satisfactory for the production of castings. Manganese is frequently added to these alloys for the purpose of improving their corrosion resistance, but it does not affect their casting quality to any substantial degree. Where attempts have been made to hot work these same alloys in the production of wrought articles, it has been found that the best workability is obtained by limiting the aluminum content to less than about 3 per cent. However, alloys containing 5 per cent or more aluminum have a higher strength and consequently are desired for many applications. Also, as the aluminum content of these alloys is increased, they become more difficult to work, especially at elevated temperatures, because of the tendency of the billets to crack when pressed, rolled, or forged. 10 In order to successfully fabricate the alloys containing more than 5 per cent aluminum it has been necessary to exercise rigid control over the heating and working conditions. In other words, the attainment of high strength in alloys of the foregoing type is achieved at the expense of ease 15 in hot working.

In the production of wrought articles, the major portion of the reduction or change in shape is accomplished at an elevated temperature where 20 the metal is much more plastic than at ordinary temperatures. As a matter of practice the deformation of the metal is performed well above the temperature at which strains would be developed of the character found in the cold worked product. In the fabrication of magnesium base alloys hot working is usually done above about 25 600° Fahrenheit. At this and higher temperatures the alloys are readily shaped without leaving deleterious residual strains. Although the 30 alloy becomes sufficiently plastic at these temperatures to be easily deformed, it may lose its cohesive quality to such an extent that cracks or incipient fractures are created under pressure of the hammer, roll, or plunger, which prevent it 35 from being utilized in the subsequent manufacture of wrought articles. Some alloys are more prone to exhibit this behavior than others. Magnesium base alloys containing from about 5 to 10 per cent aluminum, 0.1 to 1 per cent manganese, 0.05 to 0.5 40 per cent calcium, and 0.1 to 1.5 per cent zinc

belong to this group which in terms of the art are called hot short. Particular pains must therefore be taken to avoid the formation of cracks with a consequent increase in cost of production.

My invention is directed toward overcoming the disadvantages enumerated hereinabove with respect to the hot working of magnesium-aluminum-manganese-zinc-calcium alloys. In particular, it is an object of my invention to improve 10 the ductility of these alloys at elevated temperatures without detracting from their strength or other desirable properties. I have discovered that magnesium-aluminum-manganese-zinc-calcium alloys can be rendered more ductile under 15 the conditions imposed by working at high temperatures, such as have been referred to above, by the addition of a small amount of lead amounting to from 0.1 to 1 per cent of the total weight 20 of the alloy. I have found, in addition, that this alloying constituent does not substantially change or affect other desirable properties of the base alloy, but only effects a remarkable and beneficial change in its working characteristics at elevated temperatures. Further, I have determined 25 that the hot working properties of magnesium-aluminum-manganese-zinc-calcium alloys can be similarly improved by incorporating in the alloy an amount of thallium and cadmium varying in amount from 0.1 to 1 per cent of the 30 total weight of the alloy. My improved alloys containing the metals lead, thallium, and cadmium, individually or collectively in combination, within the amounts set forth, show a pronounced 35 beneficial effect during hot working, which is surprising in view of the small amount of the alloying constituent employed. If used in combination, the total amount should not exceed 2 per cent. The operation of hot working of this 40 type of base alloy is simply and economically expedited by the use of these improved alloys.

The operation of my invention is well exemplified by the following test which has been found to indicate the relative capacity of different alloys for being hot worked. The test comprises heating test bars mounted in a fixture to a predetermined temperature, immediately fastening the bar and fixture to a pendulum, and causing the pendulum to swing so that a cross member of the fixture encounters a stop on the frame of the 45 machine with the resultant breaking of the bar in tension on impact. The elongation of the 50 broken test piece is then measured, the alloy having the greatest elongation under the impact being considered the most ductile and susceptible 55

to hot working without exhibiting cracks. An exceptionally high correlation has been established between the results of this test and the actual behavior of alloys when rolled, extruded, 5 pressed, or forged. The test has therefore come to be treated as a reliable guide in ascertaining the relative workability of different alloys at elevated temperatures.

The effect of lead, thallium, and cadmium is 10 illustrated in alloys of the composition indicated below which were extruded and heated to a temperature of 550° Fahrenheit, 600° Fahrenheit, the practicable minimum hot working temperature, 15 650° Fahrenheit, and 700° Fahrenheit, and broken in tension under impact. The temperature to 20 which the particular bars were heated and the elongation of the broken test pieces are also shown in the table below.

| 20 | Composition |     |     |     |     |     | Per cent elongation in 2" at |         |         |         |         |
|----|-------------|-----|-----|-----|-----|-----|------------------------------|---------|---------|---------|---------|
|    | Al          | Zn  | Mn  | Ca  | Pb  | Tl  | Cd                           | 550° F. | 600° F. | 650° F. | 700° F. |
| 25 | 6.5         | 0.5 | 0.3 | 0.1 | —   | —   | —                            | 27.6    | 22.5    | 10.0    | —       |
|    | 6.5         | 0.5 | 0.3 | 0.1 | 0.3 | —   | —                            | 34.0    | 41.1    | 39.1    | 12.5    |
|    | 6.5         | 0.5 | 0.3 | 0.1 | 0.5 | —   | —                            | 30.2    | 47.1    | 16.3    | 10.0    |
|    | 6.5         | 0.5 | 0.3 | 0.1 | 0.7 | —   | —                            | 32.0    | 31.8    | 26.2    | 15.7    |
|    | 6.5         | 0.5 | 0.3 | 0.1 | —   | 0.5 | —                            | 35.7    | 40.2    | 36.5    | 22.2    |
|    | 6.5         | 0.5 | 0.3 | 0.1 | —   | —   | 0.5                          | 35.3    | 39.8    | 39.8    | 12.4    |

30 From the foregoing data it is at once apparent that the elongation of the basic magnesium-aluminum-zinc-manganese-calcium alloy decreases rapidly above 600° Fahrenheit, whereas the alloys containing lead, thallium, or cadmium 35 show a much lower diminution in this property with a rise in temperature above 600° Fahrenheit. Furthermore, it is to be observed that the latter alloys show a better ductility at all the temperatures than does the normal product.

While magnesium base alloys composed of magnesium, from about 5 to 10 per cent aluminum, 0.1 to 1 per cent manganese, 0.05 to 0.5 per cent calcium, 0.1 to 1.5 per cent zinc, and 0.1 to 1 per cent of at least one of the group 5 of elements lead, thallium, and cadmium, may be satisfactorily hot worked; I have found that those alloys which are composed of magnesium, from about 6 to 9 per cent aluminum, 0.2 to 0.6 per cent manganese, 0.05 to 0.25 per cent calcium, 10 0.1 to 1.3 per cent zinc, and 0.2 to 0.75 per cent of at least one of the metals lead, thallium, and cadmium are particularly desirable in making 15 wrought articles.

The alloy may be produced in any suitable 15 manner. I prefer, however, to add the heavy low melting point metals to the melt in elemental form, stirring the liquid bath sufficiently to prevent segregation or settling of the added substance. 20

I claim:

1. A magnesium base alloy containing from 5 to 10 per cent aluminum, 0.1 to 1 per cent manganese, 0.1 to 1.5 per cent zinc, 0.05 to 0.5 per cent calcium, and 0.1 to 1 per cent lead, 25 and characterized by improved ductility and freedom from hot-shortness under mechanical deformation at elevated temperatures.

2. A magnesium base alloy composed of from 6 to 9 per cent aluminum, 0.2 to 0.6 per cent manganese, 0.1 to 1.3 per cent zinc, 0.05 to 0.25 per cent calcium, and 0.2 to 0.75 per cent lead, 30 the balance being magnesium.

3. A magnesium base alloy composed of 6.5 per cent aluminum, 0.5 per cent zinc, 0.3 per 35 cent manganese, 0.1 per cent calcium, and 0.3 to 0.7 per cent lead, the balance being magnesium.

EDWARD F. FISCHER.

CERTIFICATE OF CORRECTION.

Patent No. 2,095,975.

October 19, 1937.

EDWARD F. FISCHER.

It is hereby certified that error appears in the printed specification of the above numbered patent requiring correction as follows: Page 1, first column, line 5, for "0.05" second occurrence, read 0.5; and that the said Letters Patent should be read with this correction therein that the same may conform to the record of the case in the Patent Office.

Signed and sealed this 16th day of November, A. D. 1937.

(Seal)

Henry Van Arsdale,  
Acting Commissioner of Patents.

to hot working without exhibiting cracks. An exceptionally high correlation has been established between the results of this test and the actual behavior of alloys when rolled, extruded, 5 pressed, or forged. The test has therefore come to be treated as a reliable guide in ascertaining the relative workability of different alloys at elevated temperatures.

The effect of lead, thallium, and cadmium is 10 illustrated in alloys of the composition indicated below which were extruded and heated to a temperature of 550° Fahrenheit, 600° Fahrenheit, the practicable minimum hot working temperature, 15 650° Fahrenheit, and 700° Fahrenheit, and broken in tension under impact. The temperature to 20 which the particular bars were heated and the elongation of the broken test pieces are also shown in the table below.

| 20 | Composition |     |     |     |     |     | Per cent elongation in 2" at |         |         |         |         |
|----|-------------|-----|-----|-----|-----|-----|------------------------------|---------|---------|---------|---------|
|    | Al          | Zn  | Mn  | Ca  | Pb  | Tl  | Cd                           | 550° F. | 600° F. | 650° F. | 700° F. |
| 25 | 6.5         | 0.5 | 0.3 | 0.1 | —   | —   | —                            | 27.6    | 22.5    | 10.0    | —       |
|    | 6.5         | 0.5 | 0.3 | 0.1 | 0.3 | —   | —                            | 34.0    | 41.1    | 39.1    | 12.5    |
|    | 6.5         | 0.5 | 0.3 | 0.1 | 0.5 | —   | —                            | 30.2    | 47.1    | 16.3    | 10.0    |
|    | 6.5         | 0.5 | 0.3 | 0.1 | 0.7 | —   | —                            | 32.0    | 31.8    | 26.2    | 15.7    |
|    | 6.5         | 0.5 | 0.3 | 0.1 | —   | 0.5 | —                            | 35.7    | 40.2    | 36.5    | 22.2    |
|    | 6.5         | 0.5 | 0.3 | 0.1 | —   | —   | 0.5                          | 35.3    | 39.8    | 39.8    | 12.4    |

30 From the foregoing data it is at once apparent that the elongation of the basic magnesium-aluminum-zinc-manganese-calcium alloy decreases rapidly above 600° Fahrenheit, whereas the alloys containing lead, thallium, or cadmium 35 show a much lower diminution in this property with a rise in temperature above 600° Fahrenheit. Furthermore, it is to be observed that the latter alloys show a better ductility at all the temperatures than does the normal product.

While magnesium base alloys composed of magnesium, from about 5 to 10 per cent aluminum, 0.1 to 1 per cent manganese, 0.05 to 0.5 per cent calcium, 0.1 to 1.5 per cent zinc, and 0.1 to 1 per cent of at least one of the group 5 of elements lead, thallium, and cadmium, may be satisfactorily hot worked; I have found that those alloys which are composed of magnesium, from about 6 to 9 per cent aluminum, 0.2 to 0.6 per cent manganese, 0.05 to 0.25 per cent calcium, 10 0.1 to 1.3 per cent zinc, and 0.2 to 0.75 per cent of at least one of the metals lead, thallium, and cadmium are particularly desirable in making 15 wrought articles.

The alloy may be produced in any suitable 15 manner. I prefer, however, to add the heavy low melting point metals to the melt in elemental form, stirring the liquid bath sufficiently to prevent segregation or settling of the added substance. 20

I claim:

1. A magnesium base alloy containing from 5 to 10 per cent aluminum, 0.1 to 1 per cent manganese, 0.1 to 1.5 per cent zinc, 0.05 to 0.5 per cent calcium, and 0.1 to 1 per cent lead, 25 and characterized by improved ductility and freedom from hot-shortness under mechanical deformation at elevated temperatures.

2. A magnesium base alloy composed of from 6 to 9 per cent aluminum, 0.2 to 0.6 per cent manganese, 0.1 to 1.3 per cent zinc, 0.05 to 0.25 per cent calcium, and 0.2 to 0.75 per cent lead, 30 the balance being magnesium.

3. A magnesium base alloy composed of 6.5 per cent aluminum, 0.5 per cent zinc, 0.3 per 35 cent manganese, 0.1 per cent calcium, and 0.3 to 0.7 per cent lead, the balance being magnesium.

EDWARD F. FISCHER.

CERTIFICATE OF CORRECTION.

Patent No. 2,095,975.

October 19, 1937.

EDWARD F. FISCHER.

It is hereby certified that error appears in the printed specification of the above numbered patent requiring correction as follows: Page 1, first column, line 5, for "0.05" second occurrence, read 0.5; and that the said Letters Patent should be read with this correction therein that the same may conform to the record of the case in the Patent Office.

Signed and sealed this 16th day of November, A. D. 1937.

(Seal)

Henry Van Arsdale,  
Acting Commissioner of Patents.

CERTIFICATE OF CORRECTION.

Patent No. 2,095,975.

October 19, 1937.

EDWARD F. FISCHER.

It is hereby certified that error appears in the printed specification of the above numbered patent requiring correction as follows: Page 1, first column, line 5, for "0.05" second occurrence, read 0.5; and that the said Letters Patent should be read with this correction therein that the same may conform to the record of the case in the Patent Office.

Signed and sealed this 16th day of November, A. D. 1937.

(Seal)

Henry Van Arsdale,  
Acting Commissioner of Patents.